

# United States Patent [19]

Beck

[11] 3,900,335

[45] Aug. 19, 1975

[54] PAPER SIZING

[75] Inventor: Heinz Beck, Nideggener, Germany

[73] Assignee: Akzo N.V., Arnhem, Netherlands

[22] Filed: Apr. 1, 1974

[21] Appl. No.: 456,614

[30] Foreign Application Priority Data

Apr. 14, 1973 Germany..... 2318894

[52] U.S. Cl. .... 106/213; 117/156; 162/158;  
162/175

[51] Int. Cl. .... C08b 25/02; C08b 27/52

[58] Field of Search..... 106/213; 162/158;  
260/326.5 F, 326.5 FM; 117/156

Primary Examiner—Theodore Morris  
Attorney, Agent, or Firm—Johnston, Keil, Thompson  
& Shurtliff

[57] ABSTRACT

A paper sizing agent which contains as an active sizing component at least one N,N'-alkyl-substituted aspartimide in which at least one and preferably two of the alkyl substituents consists essentially of a straight or branched alkyl chain of at least 16 carbon atoms. This aspartimide component is useful for both internal sizing or surface sizing of paper, especially paper formed of cellulosic fibers, and is readily applied as an aqueous emulsion, for example with an emulsifying agent and/or a protective colloid.

12 Claims, No Drawings

1  
PAPER SIZING

In addition to colophony (rosin), a number of other compounds have been used in the paper industry as sizing agents, including by way of example such compounds as fatty acids, fatty acid anhydrides, fatty amides, diketenes and the like. Compounds which contain acid groups precipitate as aluminum salts onto the paper fibers in the sizing procedure, for example, where aluminum is commonly present in the aqueous sizing solution as when using aluminum sulfate (alum) as a retention agent in an amount of about 0.5 to 3.0% and preferably about 1.0 to 2.0% by weight based on the paper fibers. The sizing then succeeds only at a relatively low pH-value, and these sizing agents containing acid groups therefore have a poor resistance to aging. Also, the amount of such sizing agents is relatively high, usually about 1.5 to 3% by weight with reference to the fibrous content of the paper.

Agents with an acylating or acid-reacting effect, such as fatty acid anhydrides or alkyl ketene dimers, are also disadvantageous because of their limited stability. They react not only with the hydroxyl groups of cellulosic materials but also with all other nucleophilic substances including water. For this reason, these sizing agents should not be added either at high pH-values or in the presence of aluminum sulfate at low pH-values.

For a more detailed discussion of synthetic sizing agents, attention is directed to Pulp and Paper Manufacture, edited by MacDonald and Franklin, Second Edition, Vol. III, McGraw-Hill Book Company, N.Y. (1970), pp. 50-53. This same reference also discusses surface treatments, including surface sizing, on pages 71-77, as well as internal sizing on pages 35-50. The papermaking process is generally disclosed by this reference together with suitable apparatus, including that which may be used for sizing operations. This edition is therefore incorporated hereby by reference as fully as if set forth in its entirety.

One object of the present invention is to provide a synthetic paper size or sizing agent, especially for cellulosic fibers, which overcomes the inadequacies and disadvantages of the previously used paper sizes. Another object of the invention is to provide improved paper sizing compositions and procedures capable of providing better sizing effects and/or more widely applicable sizing methods. These and other objects and advantages of the invention will become more apparent upon consideration of the following detailed specification.

It has now been found, in accordance with the present invention that one can achieve substantially improved results in the sizing of paper, especially a paper containing cellulosic fibers, by an addition to the paper of a synthetic sizing agent in which the essential active component is an N,N'-alkyl-substituted aspartimide in which at least one alkyl substituent consists essentially of an alkyl chain of at least 16 carbon atoms and preferably about 18 to 40 carbon atoms. Other than the succinimido group itself



## 2

which may be present once or twice, the aspartimide compounds of the invention may contain a total of about 18 to 104 carbon atoms, preferably about 40 to 80 carbon atoms, in the alkyl chain or chains. Although the alkyl chain is preferably a straight chain of essentially saturated hydrocarbon structure, it may be a branched chain and it may also be interrupted by one or two hetero atoms such as nitrogen, oxygen or sulfur. The alkyl chain may also contain one or two functional groups, especially a primary, secondary or tertiary amino group. Other functional groups include hydroxyl, ether, ester, carboxyl or carbonyl groups. Also included are sulfur-derivatives such as thioether, thioester and sulfonic or sulfonyl groups. The presence of one or two such hetero atoms or functional groups in the alkyl chain or chains can be tolerated without departing substantially from the essential hydrocarbon structure of these chains and without impairing the paper sizing properties of the N,N'-alkyl-substituted aspartimide compounds.

The intentional inclusion of such hetero atoms and especially the functional groups is of particular advantage for the purpose of providing especially compatible compositions for paper treatment where similar long chain alkyl-substituted compounds may be used as surface active agents in the sizing operation or in previous or subsequent treatments of the paper. Moreover, minor variations in the properties of the sized paper can be achieved with an otherwise closely related class of sizing agents based upon the essential disubstituted aspartimide structure.

A single generic structural formula cannot be given which will include a number of suitable variations of the aspartimide compounds, and in some instances it is easier to provide a mixture of these sizing agents rather than a single compound.

However, the N,N'-alkyl-substituted aspartimides of the present invention, sometimes referred to as "asparaginimides" may be generally illustrated by the structural formula



wherein R<sub>1</sub> and R<sub>2</sub> each preferably represent a long chain alkyl group of at least 16 and preferably about 18 to 24 carbon atoms. It is also feasible, however, to provide somewhat more complex tertiary amino compounds represented by the formula



wherein R<sub>1</sub> and R<sub>2</sub> have the same meaning given above while R' is hydrogen, R<sub>1</sub> or another radical

3



with  $R_1$  and  $R_2$  again having the same meaning given above.

Two succinimido groups may also be joined by an alkylene bridge between the imido nitrogen atom as represented by the formula



where  $R''$  is hydrogen or  $R_1$  and  $m$  is an integer of 2 up to about 8, preferably 3 to 6, and  $R_1$  is again a long chain alkyl group.

Still another representative class of aspartimide compounds may be illustrated by the formula



wherein  $R_2$  is the long chain alkyl group and  $m$  is an integer of 2 to 8, preferably 3 to 6.

In all of the noted formulae, it will be understood that the alkyl chain may contain hetero atoms and/or functional groups as described above, i.e., so that  $R_1$  and  $R_2$  may be further defined as being long chain radicals of the formulae

$-(CH_2)_n-R$

or



in which:

$n$  is a whole integer of at least 2,

$R$  is hydrogen, alkyl, alkoxy, alkoxyalkyl, hydroxy, hydroxylalkyl, hydroxylalkoxyalkyl, thioalkoxy, alkanoyl, alkoxycarbonyl, and alkylcarboxamido or alkylamidocarbonyl; and

$R_3$  and  $R_4$  each represent hydrogen, alkyl, hydroxylalkyl, alkoxyalkyl or alkyl substituted by a terminal carboxylic acid or its alkyl ester, provided however that each long chain radical must contain a total of at least 16 carbon atoms and preferably about 18 up to 40 carbon atoms.

Thus, in addition to the preferred hetero atoms  $-N-$ ,  $-O-$  and  $-S-$  as bridging groups, these long chain radicals may also contain other functional bridging groups such as

4



5 or the methylene bridge



in which  $Y$  is hydrogen, alkyl, hydroxy or even other functional substituents which are essentially inert under a wide range of sizing conditions and up to temperatures of about 200°C.

In general, it is preferable to employ those long chain radicals which are derived from readily available aliphatic amines, especially saturated fatty amines, butu also diamines and polyalkylpolyamines.

The  $N,N'$ -alkyl-substituted aspartimides can be easily obtained by melting together at least one amine and maleic acid anhydride or the lower alkyl esters of maleic or fumaric acid, followed by heating for a short period of time, e.g., up to one hour, at a temperature of about 150°C. to 200°C. In general, the reaction product may be used directly in its crude form without purification, or it may be recrystallized from a suitable solvent such as acetone.

By way of example, the following types of amines can be identified as being especially suitable for the preparation of the desired aspartimide compounds. Where the compound is defined by a number, this is its Registry No. see Chemical Abstracts Index, 1967-1971, Vols. 66-75.

1. Alkylamines, for example:

Hexadecylamine

Octadecylamine

Eicosylamine

Docosylamine

Tetracosylaminoo

(These amines or their mixtures are commercially available.)

2. Alkylamines containing an imino ( $-NH-$ ) bridge in the carbon chain, for example compounds of the formula



wherein  $a$  is a small whole integer of about 2 to 6, preferably 2 or 3,  $R$  preferably being an alkyl chain of  $C_{14}H_{29}$  to  $C_{24}H_{49}$ .

3. Alkylamines containing a tertiary nitrogen atom in the chain, for example compounds of the formula:



wherein  $a$  has the meaning previously given and  $R$  is preferably an alkyl chain of about  $C_6H_{13}$  to  $C_{24}H_{49}$ . Examples of such compounds are:

$N,N$ -ditetradecylethylenediamine-1,2

$N,N$ -dihexadecylpropylenediamine-1,3

$N,N$ -dioctadecylpropylenediamine-1,3

$N,N$ -diethylhexamethylenediamine-1,6

4. Amines with an oxygen ( $-O-$ ) bridge in the carbon chain of the formula



wherein  $a$  has the meaning previously given, especially 2 to 3, and  $R$  is an alkyl chain of about  $C_{14}H_{29}$  to  $C_{32}H_{65}$ . Examples of such compounds are:

- 3-octadecyloxypropylamine (No. 7617-75-6)  
3-hexadecyloxypropylamine (No. 4673-33-0).

5. Amines with a sulfur ( $-S-$ ) bridge in the carbon chain of the formula



wherein  $a$  has the meaning previously given, especially 2 or 3, and  $R$  is again preferably  $C_{14}H_{29}$  to  $C_{32}H_{65}$ .<sup>10</sup>

\* Examples of such compounds are: Dodecylthiopropylamine (No. 2g873-33-4) Tetradecylthiopropylamine (No. 2g873-32-3)

6. Amines containing an ester group in the carbon chain, for example of the formula



wherein  $a$  is again a small whole integer of about 2 to 6, preferably 2 or 3, and  $R$  is alkyl of about  $C_8H_{17}$  to  $C_{26}H_{53}$ , preferably  $C_{13}H_{27}$  to  $C_{17}H_{35}$ . Examples of such compounds are:



7. Amines with an amide group in the carbon chain, as represented by the formula



wherein  $a$  has the meaning previously given and  $R$  is an alkyl chain of about  $C_8H_{17}$  to  $C_{26}H_{53}$ , preferably  $C_{13}H_{27}$  to  $C_{17}H_{35}$ . Examples of these compounds are:



8. Amines which carry hydroxy groups on the carbon chain, for example:

9- or 10-hydroxyoctadecylamine (See U.S. 2,712,558)

4-amino-2-methyl-eicosanol (No. 19698-17-0)

10-amino-9-octadecanol (No. 19698-16-9)

1-amino-2,6,10,14-tetramethyl-pentadecanol-2 (No. 27885-72-9).

9. Amines which carry acid or ester groups on the carbon chain, for example:

22-amino-docosanoic acid (No. 27306-09-8)

12-amino-stearic acid (No. 30616-18-3)

2-amino-2,6,10,14-tetramethyl-pentadecanoic acid (No. 6169-48-8)

9- or 10-amino-stearic acid methyl ester (No. 29156-48-7)

6-amino-stearic acid methyl ester (No. 30616-17-2)

All of the above-noted amines represent suitable starting materials provided that there is at least one and preferably two long chains of at least 16 carbon atoms associated with one to two of the succinimido rings. However, where at least one or two of the  $R_1$  or  $R_2$  substituents represents a chain of at least 16 carbon atoms, one may also employ lower alkylamines, alkyldiamines or polyalkylenepolyamines having less than 16 carbon atoms, e.g. from 2 to 10 and preferably 2 to 6 carbon atoms, such as ethylene diamine, hexylamine, hexamethylenediamine, dipropyleneetriamine or the like. The lower alkylene diamines are of particular value in forming the bridging group  $-(\text{CH}_2)_m-$  in formulae III, IV above. Such variations are possible because the initial acid reactant, e.g., maleic acid anhydride, can first be reacted at a relatively low temperature, e.g., up to 100°C, to form an amide using one mono- or diamine reactant



followed by addition of another mono- or diamine reactant and heating at the higher recommended temperature of about 150°C to 200°C to make the addition of the amine group to the double bond and to close the imide ring.



Variations in the required temperature depend upon the initial reactants being used, and it is advisable to employ approximately stoichiometric additions at each stage of the reaction when using different amines.

Surprisingly, even mixed products or products in relatively crude form still possess good paper sizing properties within the prescribed requirement of at least one long alkyl chain substituent on the  $N,N$ -dialkylaspartamide compounds. Preferred heteroatoms or bridging groups in this alkyl chain are  $-\text{NH}-$ ,

—NR—, —O— and —CO—, where R is alkyl which may also extend up to 26 carbon atoms or more. Two or more of these bridges may be combined to yield the amide and ester groups —NHCO— or —CO—NH— and —O—CO— or —CO—O— as indicated above. Other minor variations such as the presence of one or two hydroxyl substituents or a number of lower alkyl substituents are also preferred.

Once the aspartimide compounds have been prepared, they are preferably made up in the form of aqueous emulsions for application as a paper sizing agent. Such emulsions are best produced by thorough mixing with the addition of an emulsifying agent or other components which ensure a uniform stable emulsion suitable for the treatment of paper. The emulsification of the aspartimide can thus take place in the presence of one or more of the following components:

a. An inorganic or organic acid, e.g., hydrochloric, sulfuric or phosphoric acids, or acetic, propionic or butanoic acids or longer chain alcanoic acids;

b. Cationic or nonionic emulsifiers or surface active agents of a wide variety known to be useful in paper sizing compositions and readily selected from any standard reference, e.g. quaternary alkyl ammonium chlorides such as hexadecyl- or octadecyltrimethyl ammonium chloride or the oxyethylated and/or oxypropylated polyalkylenepolyamines; and

c. Other sizing components including protective colloids, usually in the form of water-soluble or water-dispersible polymers, such as gelatin, sodium alginate, carboxymethyl cellulose (CMC), polyvinyl alcohol (PVA), or a degraded or cationic starch preparation.

Other preferred combinations of the paper sizing aspartimide compounds of the invention are those aqueous compositions which may further include one or more of the following components:

d. "Alum", the common designation for aluminum sulfate, preferably of a good commercial grade which is low in iron content; this substance being particularly useful as a complexing agent in the sizing liquor;

e. "Rosin", which consists primarily of abietic acid or closely related acids, preferably in smaller amounts as a "fortified" sizing agent, i.e., as compared to where rosin may be used alone, especially for internal sizing; with the aspartimide sizing agent, rosin can be added in preferred smaller amounts of 0.01 up to 1%, preferably about 0.1 to 0.5%, based on the fibrous content of the paper being sized;

f. Sodium aluminate ( $\text{Na}_2\text{Al}_2\text{O}_4$ ) as an extender of aluminum sulfate;

g. Wet-end additives such as polyacrylamides may also be included in small amounts;

h. Coloring agents, i.e., any compatible dyes or pigments useful for imparting color to the paper; and

i. Fillers and special fibers of all types, especially cheap materials such as calcium carbonate.

It is of particular value that one can achieve very good results in paper sizing with relatively small amounts of the aspartimide sizing agent after it has been emulsified, preferably with a cationic emulsifier, and then diluted to form a sizing liquor. In general, it is sufficient to add less than 1.5% by weight of the aspartimide sizing agent with reference to the fibrous content of the paper and very good results with internal or surface sizing can be achieved in amounts of about 0.1 to 1% by weight, preferably 0.2 to 0.8% by weight, again with reference to the dry weight of the fibers in the pa-

per. When used in combination with rosin or other sizing agents, one can use even smaller amounts of the aspartimide while also substantially reducing the required amount of the more conventional sizing agent.

It is especially surprising that the N,N-dialkyl-substituted aspartimides of the invention provide good sizing properties because other aspartic acid derivatives with similar structures exhibit no sizing activity at all or only an inconsequential sizing effect. Thus, very good sizing is obtained with N,N'-dioctadecyl-aspartimide while a similar compound, N-octadecyl-aspartic acid dioctadecyl ester exhibits no sizing activity at all. Also, melts of dioctadecylamine and maleic acid anhydride, which react without formation of the imide ring, develop only a very incomplete and unsatisfactory sizing effect.

A special advantage of the invention also resides in the fact that the aspartimide sizing agents are much more stable than the acid-forming agents. The sizing compositions can therefore be prepared as concentrates or as diluted liquors which are very stable in storage and in a wide variety of useful sizing compositions and under a wide range of sizing conditions. For example, the new sizing compositions in which the N,N'-disubstituted aspartimide is the active sizing component can be utilized in much wider pH ranges.

By comparison to rosin sizing agents, fatty acids or their anhydrides or fatty amides, the required amounts of the N,N'-disubstituted aspartimide compounds of the present invention are considerably smaller. Thus, as a general rule, it is sufficient and especially preferred to use these aspartimides in an amount of about 0.3–0.7% by weight for internal sizing and about 0.2 to 0.4% by weight for surface sizing, the percentages being with reference to the fibrous content of the paper.

The fact that these aspartimides can be applied at higher pH-values, for example at a pH of about 4.5 or more, preferably above 6, for example about 6 to 9, is of particular value in producing papers having a very good resistance to aging.

Finally, the new sizing material and the methods of application permissible therewith offer a coemployment of very inexpensive fillers such as calcium carbonate or other additives, something which cannot ordinarily be achieved with some other known natural or synthetic sizing agents.

The use of specific sizing compositions and the method of applying them to a cellulosic paper are illustrated in the following specific examples. The values given for ink resistance were determined with the aid of a "Hercules" sizing tester, explained in Hercules Bulletin PM515, using the ink test according to German Industrial Standard DIN 53 126. The time in seconds was measured up to a remission of 80%. For the Cobb-test, there was used water at 20°C. with a treatment time of one minute. The Cobb value was determined according to the method described in "TAPPI Monograph", Series No. 33 (1971), pages 108–114.

The following examples are illustrative only and are not intended as restrictions on the use of the paper sizing agent of the invention.

#### EXAMPLE 1

580 grams of N,N-dioctadecylpropylenediamine-1,3 and 86 grams of maleic acid diethyl ester were heated for one-half hour at 200°C., ethanol being distilled off.

There were formed a light colored, pasty substance which consists primarily of  $N,N'$ -bis-( $N,N$ -dioctadecylaminopropyl)-aspartimide as the desired sizing agent. It has the formula



100 grams of this substance were melted, heated up to about 100°C. and admixed under intensive stirring with a solution of 20 grams of Arquad 16/50 in 880 grams of water. (The Arquad 16/50 composition is a trademarked product obtained from Armour & Hess Ltd. and is a biodegradable cationic emulsifier consisting of a 50% solution of hexadecyltrimethylammonium chloride in isopropanol). The resulting emulsion was sent through a flask homogenizer while hot at about 300 atm. gauge. From this original emulsion, an aqueous sizing liquor was produced which contained 4% by weight of degraded starch in addition to 0.3% by weight of the active sizing agent.

A neutral paper of 70 g/m<sup>2</sup> in weight per unit area was selected for sizing, the paper being produced from 70% coniferous cellulose sulfite pulp and 30% beechwood cellulose sulfite pulp and 40° SR (the Schopper-Riegler degree of freeness of the pulp). This paper was surface sized on a conventional sizing press with the sizing liquor with an approximately 100% by weight absorption of the liquor by the paper. Accordingly, the sized paper contained about 0.3% by weight of the active sizing substance besides the starch, taken with reference to the cellulosic fibers. The sized paper, after drying, exhibited an ink resistance of 1.949 sec. and a Cobb value of 21.4.

#### EXAMPLE 2

The aspartimide obtained in Example 1 was again made up into an emulsion in the same manner except that the solution added to make up the original emulsion contained 20 grams of a cationic starch. The surface sizing was carried out exactly as in Example 1 and resulted in a paper with an ink resistance of 1.726 sec. and a Cobb value of 19.2.

#### EXAMPLE 3

The aspartimide obtained in Example 1 was again emulsified as described therein except that 15 grams of acetic acid were also present in the aqueous solution used for the emulsification besides the cationic emulsifier (Arquad 16/50). The surface sizing was carried out as in Example 1 to yield a paper with an ink resistance of 1.102 sec. and a Cobb value of 20.0.

#### EXAMPLE 4

2 mols of octadecylamine were melted together with 1 mol of maleic acid anhydride and heated at 180°–200°C. for one-half hour. The solidified melt which consisted primarily of  $N,N'$ -dioctadecylaspartimide having the formula



was emulsified as in Example 1 and then made up into an aqueous sizing liquor and applied to the paper exactly as described in Example 1. In this case, a paper was obtained with an ink resistance of 1.048 sec. and a Cobb value of 19.2.

#### EXAMPLE 5

The surface sizing described in Example 4 was carried out with the aspartimide sizing agent as described therein but using a paper which differed from Example 4 in that it contained sufficient aluminum sulfate to yield a pH-value of 4.5. The sized paper exhibited an ink resistance of 2.934 sec. and a Cobb value of 16.8.

#### EXAMPLE 6

In a paper machine type "Kaumuerer" used for testing purposes, there was processed a neutral pulp of 70% coniferous cellulose sulfite pulp and 30% beechwood cellulose sulfite pulp of 42°SR while adding the emulsion according to Example 4 such that there was incorporated 0.5% by weight of the aspartimide sizing agent as well as 0.3% by weight of Kymene as a retention agent, calculated with reference to the cellulosic fibers, thereby obtaining a sized paper of a weight per unit area of 70 g/m<sup>2</sup>. (The Kymene substance is a trademarked product of Hercules Powder, Inc. and is a reaction product of adipic acid, polyalkylenepolyamine and epichlorhydrin.)

The sized paper product in this case had an ink resistance of 766 sec. and a Cobb value of 25.6.

#### EXAMPLE 7

3 mols of octadecylamine were melted together with 2 mols of maleic acid anhydride and heated for one-half hour at a temperature of 180°–200°C. The elementary analysis of the melt recrystallized from acetone identified the composition as being that of  $N,N$ -di-( $N$ -octadecylsuccinimido)-octadecylamine having the formula



The crude melt was emulsified as in Example 1. It was then added as a sizing agent to the pulp as in Example 6. The resulting paper had an ink resistance of 2.000 sec. and a Cobb value of 21.0.

#### EXAMPLE 8

1 mol of  $N,N$ -dioctadecylpropylenediamine-1,3 was melted together with 1 mol of maleic acid anhydride at the lowest possible temperature. Into this melt, there was introduced 0.5 mols of 1,6-diaminohexane, and the mixture was then heated for one-half hour at 180°–200°C. The resulting composition was identified by elementary analysis as being that of  $N,N'$ -bis-

(dioctadecylaminopropylsuccinimido)-1,6-diaminohexane of the formula



it being understood that the reaction product may also contain some N-monosubstituted compounds which also fall within the scope of the invention.

The melt of this mixture was emulsified as in Example 1 and was then added as a sizing agent to the pulp as in Example 6. The internally sized paper product had an ink resistance of 900 sec. and a Cobb value of 19.0.

The invention is hereby claimed as follows:

1. A stable sizing agent for paper comprising:
  - a. water;
  - b. an emulsifying agent; and
  - c. as the active sizing component an N,N'-alkyl-substituted aspartimide in which at least one alkyl substituent consists essentially of an alkyl chain of at least 16 up to about 40 carbon atoms.
2. A sizing agent as claimed in claim 1 wherein said alkyl chain contains about 18 to 40 carbon atoms.

3. A sizing agent as claimed in claim 1 wherein said alkyl chain is interrupted by one to two hetero atoms selected from the group consisting of nitrogen, oxygen and sulfur.

5. A sizing agent as claimed in claim 1 wherein said alkyl chain contains from one to two functional groups selected from the class consisting of amino, hydroxy, ether, ester, carboxyl, carbonyl, thioether, thioester and sulfono groups.

10. 5. A sizing agent as claimed in claim 1 wherein the emulsifying agent is a surface active cationic or non-ionic emulsifier.

6. A sizing agent as claimed in claim 1 in further combination with a protective colloid.

15. 7. A sizing agent as claimed in claim 1 in further combination with a degraded or cationic starch as an additional sizing component.

8. A sizing agent as claimed in claim 1 containing an inorganic or organic acid.

20. 9. A sizing agent as claimed in claim 1 applied to a cellulosic paper product as an internal or surface sizing.

10. A method of sizing paper which comprises applying to a fibrous paper material a sizing composition containing water, an emulsifying agent and as the active sizing component an N,N'-alkyl-substituted aspartimide in which at least one alkyl substituent consists essentially of at least 16 up to about 40 carbon atoms.

11. A method as claimed in claim 10 wherein said sizing composition is applied at a pH-value above 4.5.

30. 12. A method as claimed in claim 11 wherein said sizing composition is applied at a pH-value of about 6 to 9.

\* \* \* \* \*

35

40

45

50

55

60

65